

## UNITED STATES PATENT OFFICE.

GEORGE L. SCHWARTZ, OF WILMINGTON, DELAWARE, ASSIGNOR TO E. I. DU PONT DE NEMOURS & COMPANY, OF WILMINGTON, DELAWARE, A CORPORATION OF DELAWARE.

## CELLULOSE-ESTER COMPOSITION.

No Drawing.

Application filed June 15, 1923. Serial No. 645,677.

This invention relates to cellulose ester compositions, and particularly pyroxylin coating compositions, and comprises, as new products, combinations of cellulose esters (cellulose acetate, cellulose nitrate, etc.) with mixed esters (and specifically mixed glycerides) of the lower and higher fatty acids.

The main object of my invention is to provide a pyroxylin softener which can be used to advantage in place of the castor oil which usually functions as the softener at the present time in pyroxylin coating compositions.

Another object of my invention is to provide a new, odorless artificial leather.

The new softeners, which are preferably mixed glycerides of coconut oil acids and acetic acid, are described and claimed in my copending application, Serial No. 551,734 filed April 11, 1922, Patent No. 1,558,299 of Oct. 20, 1925. In the present case I claim the combination of these new substances with cellulose esters (and particularly with nitrocellulose) to form new and valuable coating compositions.

The vegetable oils have long been used as softeners of pyroxylin, and in particular castor oil and blown rapeseed oil have been used. Both of these oils are glycerides of unsaturated fatty acids. Their iodine numbers are high, and probably as a result of this unsaturated condition they are subject to certain physical or chemical changes. For example, castor oil readily becomes rancid when exposed in a pyroxylin film, and it gradually undergoes oxidation which causes a hardening of the film. Practically the only low melting vegetable oil that does not have a high iodine number is coconut oil. This oil is available in large quantities and would be an excellent softener of pyroxylin if its melting point were somewhat lower. It is much less subject to rancidity development and to gradual oxidation than oils now used, because the percentage of unsaturated glycerides which it contains is very low.

I have found that it is often desirable to use as a softener a substance which has mild solvent power for pyroxylin. All of the known vegetable oils are practically

without solvent action on pyroxylin, and it has heretofore been thought necessary, if solvent power was required, to add a solvent softener to the vegetable oil.

I have discovered that if an acyl group of a lower fatty acid is introduced into one or more of the glycerides of coconut oil, or of various other vegetable oils, the solvent power of the resulting glyceride for pyroxylin is appreciably increased, while at the same time the freezing point of the glyceride is lowered. This lowering of the freezing point is sometimes quite marked. Commercial coconut oil, for example, has a freezing point of from 14 to 22° C., whereas, after the introduction of an acetyl group to form a mixed ester, the melting point is usually between -5 and -13° C., the exact value depending upon the extent to which the acetyl group has displaced higher fatty acid radicals in the glycerides present. In general a mixed glyceride made in accordance with my process should have a freezing point below 10° C., especially where the mixed glyceride is to be used as a softener of pyroxylin, although in some cases the increase in solvent power attending the introduction of a lower fatty acid radical may be so great as to render the glyceride suitable as a softener even though the freezing point thereof be substantially above 10° C.

The expression "lower fatty acid" is used herein to mean either formic, acetic, or propionic, acid; and the expression "higher fatty acid" has reference to acids of the  $C_nH_{2n}O_2$  series containing more than nine carbon atoms. The alcohol radical of the mixed ester may be the radical of any one of various polyhydric alcohols, and especially of the lower polyhydric alcohols having between one and four hydroxyl groups, the principal members of this class being glycerol and ethylene, propylene, and butylene, glycols.

Where the new softener has been obtained by the action of acetic acid on coconut oil, of which the chief constituent is the glyceride of lauric acid, the new softener will consist of a mixture of mixed esters of which the major part will be acetyl-laurin, with

acetyl-palmitin and acetyl-myristin present in small proportions. The mono-acetyl-laurin formed has probably the following graphical formula:



Various alternative methods of producing 10 the new softener have been set forth in my above mentioned application, Serial No. 551,734, Patent No. 1,558,299 of Oct. 20, 1925; only my preferred method will be given herein, this method being as follows:

15 The following ingredients are mixed in a flask that is provided with a reflux condenser and are heated for 13/4 hours in an oil bath at a temperature where the acetic acid boils vigorously.

20

|                                       |      |
|---------------------------------------|------|
| Parts by weight.                      |      |
| Glycerine (containing 5% water)       | 967  |
| Glacial acetic acid (99.5% acid)      | 2250 |
| Coconut oil acids (mean mol. wt. 208) | 1560 |
| Sulfuric acid                         | 0.7  |

25 The condenser is then changed to a distilling position and as the acetic acid concentration decreases the temperature of the mixture rises and is held at 160-175° C. throughout the remaining heating period. A stream of nitrogen is passed through the mixture throughout this latter heating stage to sweep out water as formed. After neutralization is practically complete the crude

30 product is washed with an aqueous sodium chloride solution to remove sulfuric acid. The washed product is then heated for two hours on a steam bath with 2% of its weight of decolorizing carbon and is filtered. The

35 finished product obtained by carrying out this process on a small scale was a light brown, transparent, oily liquid with a slight odor resembling coconut oil and freezing at -10 to -11° C. It contained 1.03% free

40 coconut oil acids. The yield was 87.2% of the theoretical. The finished product is miscible in all proportions in mineral oil; it colloids pyroxylin at normal temperatures; and it does not become rancid.

45 A mixture of mixed glycerides prepared by the above method is practically non-volatile and cannot be distilled at pressures as low as 14 mm. without partial decomposition. This product consists of a mixture of 50 all the possible glycerides of acetic acid and coconut oil acids, ranging from some tri-acetin through the mixed glycerides to and including some coconut oil. The freezing point varies according to the ratio of acetyl to coconut oil acid groups and usually falls within the range of -5 to -13° C.

55 The coconut oil acids that I have used were obtained by hydrolysis, with subsequent distillation under reduced pressure, of commercial coconut oil.

Coconut oil, as has been indicated above, is the oil with which I prefer to start, but other materials may with advantage be converted into acetyl-glycerides in the manner above described, as, for example, commercial stearic acid, which contains a large proportion of palmitic acid, or palm kernel oil, or the acids of this oil.

60 The new softeners, when obtained from oils such as coconut oil, may be defined 75 generically as mixtures of acetyl derivatives of glycerides of two or more higher fatty acids each having from 10 to 16 carbon atoms. The glyceride mixture prepared in accordance with the above examples will contain a substantial proportion of diacetyl-glycerides of the higher fatty acids, as, for example, diacetyl-laurin, diacetyl-myristin, and diacetyl-palmitin. The molecular structure of the alpha-gamma-diacetyl-laurin, 80 which is typical, is probably as follows:



90

85 In addition to the alpha-mono-acetyl-laurin whose structure has been shown in the first of the above graphical formulas, the new softener contains the beta-mono-acetyl derivative of the various glycerides; and in addition to the alpha-gamma-diacetyl derivative, the alpha-beta-diacetyl derivative is believed to be formed, although in minor proportions.

90 An approximate idea of the relative proportions of the mixed esters of the various glycerides obtained by my process, may be gained from the following table showing the relative proportions of combined fatty acids which are present in coconut oil:

|                                                     | Per cent. |
|-----------------------------------------------------|-----------|
| Caproic ( $\text{C}_6\text{H}_{12}\text{O}_2$ )     | 0.25      |
| Caprylic ( $\text{C}_8\text{H}_{16}\text{O}_2$ )    | 0.25      |
| Capric ( $\text{C}_{10}\text{H}_{20}\text{O}_2$ )   | 19.5      |
| Lauric ( $\text{C}_{12}\text{H}_{24}\text{O}_2$ )   | 40.0      |
| Myristic ( $\text{C}_{14}\text{H}_{28}\text{O}_2$ ) | 24.0      |
| Palmitic ( $\text{C}_{16}\text{H}_{32}\text{O}_2$ ) | 10.6      |
| Oleic ( $\text{C}_{18}\text{H}_{34}\text{O}_2$ )    | 5.4       |

100 A decidedly greater lowering of the freezing point and increase in solvent power of the higher fatty acid glycerides is attained by introducing two, instead of merely one, acetyl group into the glyceride molecules. My new class of softeners includes broadly 110 both the monoacetyl-di-acyl-glycerides and the diacetyl-mono-acyl-glycerides, where "acyl" is used to mean the acid radical of a higher fatty acid, as well as corresponding glycerides containing one or two formyl, or 120 one or two propionyl, groups. These new softeners may be designated briefly as 125 "mixed glycerides".

130 This mixed glyceride is a more effective softener for pyroxylin than is castor oil, as

is indicated by the fact that a film containing pyroxylin 1 part—mixed glycerides 1 part, has about the same pliability as a film containing pyroxylin 1 part—castor oil 1.5 parts. The mixed glyceride can be used alone with nitrocellulose if the ratio of said mixed glyceride to nitrocellulose is low enough. However for fabric-coating compositions it gives the best results when mixed 10 with a lubricant such as mineral oil or esters of aliphatic alcohols with the higher fatty saturated acids such as stearic.

The following is a sample coating composition without a lubricant.

|                  | Parts. |
|------------------|--------|
| Pyroxylin        | 1.00   |
| Mixed glyceride  | 1.37   |
| Pigment          | 0.62   |
| Volatile solvent | 11.00  |

20 The following is a sample coating composition with a lubricant.

|                   | Parts. |
|-------------------|--------|
| Pyroxylin         | 1.00   |
| Mixed glyceride   | 1.34   |
| Liquid petrolatum | 0.15   |
| Pigment           | 0.62   |
| Volatile solvent  | 11.00  |

30 The ratio of mixed glyceride or a mixture of these mixed glycerides and lubricant to pyroxylin in films containing pigment can be varied from pyroxylin 1.00—softener 0.75 to pyroxylin 1.00—softener 1.62. In films containing no pigment the ratios can 35 be varied between pyroxylin 1.00—softener 0.62 to pyroxylin 1.00—softener 1.25. High ratios of softener tend to produce films too soft or sticky for good embossing and low ratios tend to produce stiff material.

40 As the volatile solvent in the above formulas there may be used a mixture containing benzene 38% and ethyl acetate 62%, or a mixture containing benzene 50%, ethyl acetate 25% and denatured alcohol 25%.

45 Many solvent mixtures other than these two may of course be used. For example, as the active solvent there may be used either acetone, acetone oils, methylacetone (a commercial mixture containing methyl acetate, methyl alcohol, and acetone), or an ether-alcohol mixture; and as the diluent there may be used, for example, ethyl alcohol, benzine or benzol.

55 The ratio of volatile solvent to non-volatile constituents may of course vary widely; thus, instead of the 11 to 3 ratio in the above formulas, the ratio of volatile solvent to nonvolatile constituents may, for example, be 18 to 3 or 21 to 3.

60 As indicated above the new nitrocellulose composition containing a mixed glyceride as the softener is especially advantageous when applied to fabrics in the manufacture of artificial leather (fabrikoid, etc.). Artificial leather containing the new nitrocel-

lulose composition is free from the objectionable odor of castor oil, and is remarkably pliable and durable.

When working with cellulose acetate the acetyl-laurins should be used in conjunction 70 with another solvent softener such as triacetin.

Where the coating composition is to be applied by calendering, and is in the form of a plastic mass, the ratio of volatile solvent 75 to non-volatile constituents may be as little as 1 to 3.

Although the mixed glycerides of higher and lower fatty acids are especially applicable as softeners of nitrocellulose in connection with the manufacture of artificial leather, they are also valuable softeners or modifiers of nitrocellulose in all of the pyroxylin industries. For example, acetyl-laurins can be used as a softener in pyroxylin 85 lacquers and enamels where it has been customary, in the past, to use castor oil. The quality of the lacquers and enamels is much improved by the use of the new softener because it is not subject to oxidation as is 90 castor oil. Acetyl-laurin may also be used as a camphor substitute in the manufacture of celluloid; it has the advantage over camphor that the product is softer and less liable to discoloration when exposed to sunlight. In fact, in any of the pyroxylin industries, where a softener or modifier has been used, the new products described will find valuable application.

I claim:

1. A composition of matter comprising nitrocellulose and a mixed ester of a lower and a higher saturated fatty acid, the alcohol radical of said ester being that of a polyhydric alcohol having between 1 and 4 105 hydroxyl groups.

2. A composition as set forth in claim 1 in which the mixed ester has a freezing point below 10° C.

3. A composition of matter comprising a 110 cellulose ester and a mixed ester of a lower saturated fatty acid and a higher saturated fatty acid having from 10 to 16 carbon atoms, the alcohol radical of said ester being that of a polyhydric alcohol having between 1 and 4 hydroxyl groups.

4. A composition of matter comprising a cellulose ester and a mixed glyceride of a lower saturated fatty acid and a higher saturated fatty acid having from 10 to 16 carbon atoms. 120

5. A composition of matter comprising a cellulose ester and a mixed glyceride of a lower saturated fatty acid and a higher saturated fatty acid having from 10 to 16 carbon atoms, the glyceride having a freezing point below 10° C. 125

6. A composition of matter comprising nitrocellulose and a mixed glyceride of a lower and a higher saturated fatty acid. 130

7. A coating composition comprising a mixture of pyroxylin and a softener consisting of a mixed glyceride of a lower and a higher saturated fatty acid.
- 5 8. A coating composition comprising pyroxylin and a mixed glyceride of acetic acid and a higher saturated fatty acid.
9. A coating composition comprising pyroxylin and a mixed glyceride of acetic acid 10 and a higher saturated fatty acid, said glyceride having a freezing point below 10° C.
10. A coating composition comprising pyroxylin and a mixed glyceride of acetic acid 15 and a higher saturated fatty acid having from 10 to 16 carbon atoms.
11. A coating composition comprising 100 parts of pyroxylin and from about 62 to 162 parts of a mixed glyceride of a lower 20 and a higher saturated fatty acid.
12. A coating composition comprising 100 parts of pyroxylin and from about 62 to 162 parts of a mixed glyceride of acetic acid and of a higher saturated fatty acid 25 whose molecular structure includes from 10 to 16 carbon atoms.
13. A coating composition comprising pyroxylin and a softener therefor consisting of an acetyl-laurin.
- 30 14. A coating composition comprising 100 parts of pyroxylin and from about 75 to 162 parts of a softener containing an acetyl-laurin.
15. A coating composition comprising nitrocellulose, a lubricant, and a mixed ester of 35 a lower and a higher fatty acid, the alcohol radical of said ester being that of a polyhydric alcohol having between 1 and 4 hydroxyl groups.
- 40 16. A coating composition comprising nitrocellulose, a lubricant, and a mixed glyceride of a lower and a higher fatty acid.
17. A coating composition comprising nitrocellulose, a lubricant, and a mixed glyceride 45 of a lower and a higher fatty acid, said mixed glyceride having a freezing point below 10° C.
18. A coating composition comprising nitrocellulose, a lubricant, and a mixed glyceride of acetic acid and of a higher fatty acid having from 50 10 to 16 carbon atoms.
19. A coating composition comprising nitrocellulose, a lubricant, and an acetyl-laurin.
- 55 20. A coating composition comprising 100 parts of nitrocellulose, from about 10 to 20 parts of a lubricant, and from about 75 to 162 parts of a mixed glyceride of acetic acid and of a higher fatty acid having from 60 10 to 16 carbon atoms.
21. A composition as set forth in claim 15 in which the lubricant is petrolatum.
22. A composition as set forth in claim 16 in which the lubricant is petrolatum.
23. A composition as set forth in claim 17 65 in which the lubricant is petrolatum.
24. A textile fabric having on one side a practically odorless pyroxylin composition containing as a softener a mixed glyceride of a lower and a higher saturated fatty acid, 70 said composition retaining its flexibility and freedom from odor for a prolonged period.
25. A pyroxylin-coated fabric in which the pyroxylin coating contains as a softener an acetyl-laurin. 75
26. A composition as set forth in claim 18 in which the lubricant is petrolatum.
27. A composition as set forth in claim 19 in which the lubricant is petrolatum.
28. A composition as set forth in claim 20 80 in which the lubricant is petrolatum.
29. A composition as set forth in claim 1 in which a pigment constitutes one component of the composition.
30. A composition as set forth in claim 4 85 in which a pigment constitutes one component of the composition.
31. A composition as set forth in claim 8 in which a pigment constitutes one component of the composition. 90
32. A composition as set forth in claim 13 in which a pigment constitutes one component of the composition.
33. A composition as set forth in claim 15 in which a pigment constitutes one component of the composition. 95
34. A composition as set forth in claim 1 which also includes a volatile solvent.
35. A composition as set forth in claim 4 which also includes a volatile solvent. 100
36. A composition as set forth in claim 9 which also includes a volatile solvent.
37. A composition as set forth in claim 13 which also includes a volatile solvent.
38. A composition as set forth in claim 15 105 which also includes a volatile solvent.
39. A composition as set forth in claim 18 which also includes a volatile solvent.
40. A composition of matter comprising a cellulose ester and a mixed ester of a lower 110 saturated fatty acid and a higher saturated fatty acid, the alcohol radical of said ester being that of a polyhydric alcohol having between 1 and 4 hydroxyl groups.
41. A composition of matter comprising a cellulose ester and a mixed glyceride of a lower saturated fatty acid and a higher saturated fatty acid. 115

In testimony whereof I affix my signature.  
GEORGE L. SCHWARTZ.